

April 13, 1943.

K. I. HARVEY

2,316,161

GRINDING TOOL

Filed May 23, 1939

15

Fig.1.



Fig.2.

18 17



Fig.3.



Fig.4.



Fig.5.

28

27

26



INVENTOR.

Kelley I. Harvey  
BY Edward Lawrence,  
his ATTORNEY.

## UNITED STATES PATENT OFFICE

2,316,161

## GRINDING TOOL

Kelsey I. Harvey, Beaver, Pa.

Application May 23, 1939, Serial No. 275,174

14 Claims. (Cl. 51—307)

This invention relates generally to abrading and more specifically to abrading tools, their composition and the method of making the same.

The principal object of this invention is the provision of a novel abrading composition and the method of making the same.

Another object is the provision of an abrading composition having a metal reenforcing or supporting insert.

Another object is the provision of a novel abrading composition wherein the coefficient of the bond is such that it will fracture during use, thereby exposing the grit to produce faster and cooler abrading.

Another object is the provision of an abrading composition wherein the proportion of the grit materially exceeds that of the bond after it has been heat treated as compared with known types of abrading compositions known in the art.

A marked advantage is that this bonding composition may be used with any character of grit, whereas other bonds must be changed to suit the grit and the application.

Another object is the provision of a new and improved vitreous bond for uniting abrading compositions.

Another object is the provision of a novel abrading composition that may be formed, heat treated and cooled within a relatively short period of time in comparison with other brading compositions of this type known in the art.

Another object is the provision of a novel abrading composition that may be wetted for the purpose of application and immediately fired to vitrification and rapidly cooled without injury thereto.

Another object is the provision of a novel abrading composition that is capable of relatively high peripheral speeds in comparison with abrading compositions of this type known in the art.

Another object is the provision of an abrading composition that may be formed into a tool with metal embedded therein for reenforcing or supporting the tool and which may be heat treated without injury to the threads or other relatively frail portions of the metal.

Other objects and advantages appear in the following description and claims.

Innumerable abrasives have been used for many years, such as siliceous abrasives, sandstones, quartz, tripoli, pumice and volcanic dusts. These are relatively soft as compared with corundum, diamond, garnet and the artificial abrasives such as silicon carbide and fused alumina.

The latter abrasives are commonly referred to as grits and are employed in many grades as to size. These abrasives are harder and are made up in tool form with the use of a vitreous or plastic bond which unites the grit in a mass for abrading purposes. This disclosure is confined chiefly to the art of producing an abrading composition of the vitreous type including any of the above grits with an improved bond. This discovery has led to an improved abrading composition as well as to a new bond and finds a practical application in the art of abrading tools.

One outstanding characteristic of this new bond is that it may be used with any of the abrasive grits without alterations, while in most every instance in the present art the bond is not only changed for different kinds of grits but for different sizes of the same grit, such as in the production of a soft and hard abrading tool.

The preferred principal ingredients of the bond are boron, lead and lithium. The boron and the lead are preferably added in their oxide state and the lithium as a carbonate, salt or in the form of lepidolite. Granulated or powdered borax or boric acid have been found to be the best form for obtaining the boric oxide because they are comparatively less expensive than other boron compounds and they provide the boron in its oxide form which is believed to provide the best results.

Lead monoxide or litharge has been found to be the best form in which to obtain the principal ingredient lead. However red or white lead which would yield the equivalent proportion of lead monoxide may satisfactorily be used. Other forms of lead will produce good results such as lead chromate, carbonate or sulfide, but it is preferable to employ litharge.

The principal ingredient lithium may be added in the form of an oxide, a nitrate, a chloride, salt, carbonate or phosphates, but lepidolite is relatively inexpensive and may be readily obtained, which makes it a desirable form in which to obtain the lithium. Lepidolite also contains silica, alumina, potassium, fluorine and a little potash together with some lime, magnesia, rubidium oxide, calcium oxide and manganese oxide. The fluorine in this mineral is also an active fluxing agent and is believed to aid the fluxing action of the lithium. This provides another reason for preferring the use of lepidolite in place of other lithium compounds such as the lithium salts. Fluorine may be substituted for lithium in the bond but lithium is preferable.

One or more of the group including potassium,

sodium, calcium, magnesium, zinc and tin may be used individually in place of any one of the three principal ingredients in this ceramic. However, compounds of each of these elements add their singular characteristics to the composition, yet they all have about the same effect on the fusibility of the composition. Probably the most noticeable difference in the use of some of these substitutes is that they tend to make it more brittle. In some applications this may be highly desirable, whereas in others it may be preferable to maintain a softer product. Titanium, zirconium, cobalt, copper and barium have the effect of tempering the product. Some of these are too expensive to use commercially, especially in view of the beneficial results obtained with boric acid, litharge and lepidolite which are relatively cheap. However copper and barium are easily obtainable. They may be used as a substitute for one of the ingredients or they may be used in addition thereto for tempering the composition. Barium nitrate is also effective when added in the presence of lead, as the nitrate avoids the formation of metallic lead during the melting if such difficulty be experienced.

The three ingredients constituting the preferred composition of the bond, boric acid, litharge and lepidolite, were found to produce the best results when added in equal amounts by weight. However each ingredient may be used in proportions of 10% to 60% by weight to obtain the bond. These proportions may be determined by using a triaxial diagram. If other compounds containing the chemicals boron, lead and lithium are used, their proportions may be determined by setting up a triaxial diagram using the new compounds or chemicals calculated to provide approximately 15% by weight of boron, 16% by weight of lead and 6% by weight of lithium which represents the percentages of these elements when using equal proportions of boric acid, litharge and lepidolite to make up the bond. The quantity of the substitutes for lead and lithium should be determined in the same manner.

The boric acid, the litharge and the lepidolite in powdered form are thoroughly mixed together.

The size of the grit particles together with the relative grade of hardness of the tool may be determined by properly proportioning the amount of the bond of this invention to approximately the same percentages as those used by industries with the present types of bond well known in the art. The powdered bond with a sufficient amount of liquid to make it moldable, preferably water, is then added to the grit and thoroughly mixed to produce a homogeneous mass. The bond will hold the grit particles together and it is generally unnecessary to add a temporary bond such as dextrine, glutrine, glycerine or other similar ingredients.

The batch is then placed in a mold and is pressed to form the tool.

If the tool being formed is relatively large in diameter and is made with a small size grit and has a low proportion of bond, such as approximately 3%, so as to produce a soft tool, then it has been found advantageous to apply heat to the tool to initially cure the same. This preliminary heat sinters the bond at a temperature as low as 150° F. and it hardens the tool sufficiently to enable it to be handled and transported to the place of final heat treating. This feature is a very important advantage of this invention. If

a moderately sized tool, composed of approximately 10% or more bond, is being made, this preliminary heat treatment may be found unnecessary.

5      Abrasive tools may be made using from 3% to 95% by weight of bond with from 97% to 5% by weight of grit or grit and a filler-grit. The filler being such as ground quartz or other suitable material which is equally substantially inert to the fluxing action of the bond but not having the abrasive qualities of the principal grit. An increase in the percentage of the bond in a mix increases the hardness of the tool to a point commonly referred to as the saturation point beyond which an additional percentage of the bond has the tendency to decrease the hardness or cutting efficiency of the tool. This saturation point is determined by the grit, shape and size, since the surface area of the grit, that must be covered by the bond, changes in proportion to its physical characteristics. Again this bond may be successfully employed for making tools having grit sizes ranging from 8 to 600 mesh.

10     After the tool has been removed from the mold it is ready for heat treatment. Any suitable heat controlled furnace or kiln may be used for heat treating the tool. The furnace may be of the closed or open type. However a vapor is formed during the heat treating process and it will coat any exposed metal parts with a vitreous deposit which is very hard and believed to be similar to the bond. Thus it is necessary to cover the exposed portion of the metal inserts and any other metal in the furnace upon which it is not desired to have this vitreous coating.

15     A batch made up of the preferred compounds at the proportions given will sinter when heated 150° to 400° F. and becomes sticky and at about 450° to 750° F. vitrification is evident. A tool 20     heat treated at approximately 750° F. completely vitrifies in one to five hours, depending upon its mass. However it is preferable to heat treat these tools to a temperature of approximately 1300° F. to 1600° F. and have them in 25     the furnace from twenty minutes to about three hours, depending upon the mass of the tool. The temperature and the time during which it is applied is largely a matter of heat penetration and if the heat is applied locally within the mass 30     it naturally is more effective relative to the time required to treat it. The tool may then be removed as a completely heat treated article. This temperature will not produce any harmful effects on the metal inserts which are preferably 35     made of steel and the tool will be thoroughly heat treated. The tool may be removed from the furnace even though it is a cherry red color without harmful effects and placed on a suitable 40     rotary machine where any uneven or rough portions can be trimmed off, thereby trueing up the tool. Even before a tool has cooled to a degree 45     where it could not be touched by the hand it may be used for abrading purposes. These tools 50     may be heat treated at temperatures as high as 55     2500° F. as the bond has a relatively long range 60     of vitrification without harming its structure but in such cases the tool should not have any 65     metal inserts as they would burn and disintegrate.

70     If some of the elements in the above mentioned group are taken alone and used in place of lepidolite or litharge or other oxide compound, the mix will sinter at approximately 200° F. to 500° F. and the melting temperature is approximately 1000° F. to 1400° F. However the 75

substitution of these elements for boric acid produces a mix having temperature characteristics approaching that of the element added.

This bond thus provides a long range of vitrification. However when one of the elements including the group of lithium, sodium, potassium, calcium, manganese, tin, zinc and fluorine are used by themselves as an ingredient in the mix they have the tendency of shortening the range of vitrification. They may sinter at approximately the same temperature given above but vitrify at a higher temperature such as approximately 1000° F. and they may quickly liquefy. Thus it may be preferable to use an oxide, carbonate or other similar form rather than the element, depending upon the character of the tool being made.

The bond is tough and strong and can withstand severe thermal shocks. Owing to the fact that the ingredients making up this bond originally contain a considerable amount of oxygen and water by weight which are given off during the heat treating process the weight of a tool after heat treatment is materially reduced and in some instances where the bond represents a small proportion of the tool it is difficult to see it.

This bond is very tough and strong and since the elements contained therein have high fluxing characteristics it is believed to dissolve a small portion of the surface and the matrix of the grit as it vitrifies, thereby making a very strong union.

When used in abrading a small portion of the bond surrounding a piece of grit fractures and falls away, leaving a sharp edge of the grit exposed. When this sharp edge of the grit wears down or breaks off another small portion of the bond fractures and falls away, exposing a new sharp edge of the grit particle. This action produces cool clean cutting tools. This is unlike other bonds which generally release the whole grit particles when they fracture or the bond merely wears away with the grit.

Again the strength and toughness of this bond permits a tool to be used at 12,000 surface feet per minute, which is equivalent to the speed of tools made up with plastic bonds such as synthetic resins and rubber. Tools have been rotated to produce a speed as high as 16,000 surface feet per minute without breaking, whereas vitrified tools known in the art are tested at 9,500 surface feet a minute and are not recommended to be used above 7,500 surface feet a minute. It has been proven that these wheels may be safely operated at speeds equivalent to and greater than the speeds recommended for tools made with bonds comprising synthetic resins and rubber and their cool clean cutting action is maintained.

In the accompanying drawings practical embodiments illustrating the principles of this invention are shown wherein:

Fig. 1 is a sectional view showing a grinding tool having a steel reenforcing ring embedded therein.

Fig. 2 is a sectional view of a grinding tool of the disk type which may be mounted by means of independent nuts embedded in the tool and exposed on the rear face thereof.

Fig. 3 is a sectional view of a spherically shaped grinding surface tool having a reenforcing wheel formed integral with the threaded hub.

Fig. 4 is a sectional view of a small grinding tool showing a threaded metal insert in the axial center adjacent one end thereof for mounting the same.

Fig. 5 is a sectional view of a thin disk type tool with a metallic disk center.

Referring now to Fig. 1 of the drawing, 10 represents a cutting tool having a steel core member 11 with hexagonally shaped flanges 12 spaced apart, forming an annular groove 13 therebetween. The center of the core is bored out as indicated at 14 for receiving a mandrel or shaft. The bore may also be threaded as illustrated for receiving a threaded mandrel. 15 represents a reenforcing ring centrally positioned in the wheel as it is being molded.

In Fig. 2 a disk type of grinding tool 16 is shown wherein hexagonal nuts 17 are inserted in spaced relation about the tool and exposed to the rear face thereof for mounting the tool on a metal disk by means of bolts. The nuts 17 are preferably tapered on one face as illustrated at 18 so that they will resist being pulled from the sockets formed in the tool. Serrations may be formed on the surface of these metal inserts, thereby increasing their dislodging resistance.

The semi-spherically shaped tool 19 shown in Fig. 3 is provided with a hexagon shaped core 20, similar to that shown in Fig. 1 at 11, with a series of spokes 21 radiating therefrom and are connected at their outer ends by a continuous rim 22 forming a wheel. This metal insert may be made up in any desired manner. However it has been formed by welding the individual pieces together to form an integral structure.

Fig. 4 illustrates a small cylindrical tool 23 having an octagonally shaped threaded core 24 with a plurality of annular grooves 25.

In Fig. 5 the disk type tool 26 is provided with a metal disk 27 which is substantially as thin as the abrading compound on each side thereof. The metal disk is preferably made integral with the metal core 28. In this manner a large diameter tool may be made up with a very fine grit in a vitreous bonding abrading compound.

The shape of these mounting and reenforcing inserts may be formed to best serve the purpose for which the tool is intended and their limitations are incalculable. However this improved abrading composition provides a vitreous bond which surpasses other abrading tools of similar character and permits the use of metal inserts which cannot be embodied in tools requiring heat treatment at temperatures at which metals, such as steel, are impaired or become distorted. Again this same abrading composition may be heat treated at higher temperatures, in which case the metal inserts are omitted, without detracting from the abrading characteristics and without requiring the slow cooling or annealing of the tools for periods of ten days to three weeks, as in the present practice.

In filling the molds the material is preferably introduced in a whirling or spinning manner.

Another important improvement comprising this invention lies in the fact that the principal ingredients which are mixed together to produce this bond are initially in the form of oxides of the separate elements the greater proportion of the weight of which is driven off by the vitrification. For example a bond mix initially made of equal proportions of boric acid, litharge and lepidolite is believed to lose approximately one-third of its weight upon vitrification.

Thus when the tool is pressed there is sufficient bulk in the bond to provide "green strength" and after heat treatment the bond having been materially reduced provides a cool free cutting tool open in structure.

Again if a batch is placed in a mold and is heated prior to or simultaneously with the application of pressure for forming the tool it is obvious that a portion of the volatile matter of the bond may be permitted to escape before the tool is fully pressed or formed. By thus regulating the loss of the volatile matter the density or the open porosity of the tool may be determined. This process may be advantageously employed in place of the use of fillers for regulating the density in a tool. It also provides a method for obtaining tools of greater density with the use of materially reduced pressures.

I claim:

1. An abrasive article consisting of abrasive particles bonded with a ceramic derived of a boron salt, a lead salt and a lithium salt.

2. An abrasive article consisting of abrasive grains bonded with a ceramic composition consisting of a boron salt, a lead salt and a lithium salt, wherein the boron and lead were initially approximately from 4 to 30 percent by weight of the salt and the lithium from 1.5 to 11 percent by weight of the salt.

3. An abrasive article consisting by weight of from 70 to 97 percent of an abrasive material bonded with a fused ceramic composition initially by weight of from 30 to 3 percent, the ceramic bond consisting of a boron salt, a lead salt and a lithium salt, wherein the boron and lead were initially approximately from 4 to 30 percent by weight of the salt and the lithium from 1.5 to 11 percent by weight of the salt.

4. An abrasive article consisting by weight of from 97 to 5 percent of an abrasive grit and a grit filler bonded with a fused ceramic composition initially by weight of from 3 to 95 percent, the ceramic bond consisting of a boron salt, a lead salt and a lithium salt, wherein the boron and lead were initially approximately from 4 to 30 percent by weight of the salt and lithium from 1.5 to 11 percent by weight of the salt.

5. An abrasive article consisting of abrasive particles bonded with a complex ceramic containing substantial proportions of boron, lead and lithium substances.

6. An abrasive charge for the production of abrasive articles consisting of abrasive particles, and a complex ceramic bond of 10% to 60% of boron containing substance, 10% to 60% of lead

containing substance, and 10% to 60% of lithium containing substance.

7. An abrasive charge for the production of abrasive articles consisting of abrasive particles, and a complex ceramic bond of boric oxide, lead oxide, and a lithium containing substance initially in approximately equal proportions.

8. An abrasive article consisting of abrasive particles bonded with a ceramic containing substantial proportions of boron, lead, lithium and a substance containing one of a group consisting of potassium, sodium, calcium, magnesium, zinc and tin.

9. An abrasive article consisting of abrasive particles bonded with a ceramic containing substantial proportions of boron, lithium and a substance containing one of a group consisting of potassium, sodium, calcium, magnesium, zinc and tin.

10. An abrasive article consisting of abrasive particles bonded with a ceramic containing substantial proportions of lead, a lithium and a substance containing one of a group consisting of potassium, sodium, calcium, magnesium, zinc and tin.

11. An abrasive article consisting of 70% to 99.1% abrasive particles and 30% to .9% of a ceramic bond, of boron, lithium, and a substance containing one of a group consisting of potassium, sodium, calcium, magnesium, zinc and tin.

12. An abrasive article of the character described consisting of abrasive particles and a ceramic bond comprising boron, lead, lithium substances, in proportions approximately providing 15 parts by weight of boron, 16 parts by weight of lead, and 6 parts by weight of lithium.

13. An abrasive article of the character described consisting of abrasive particles bonded with a fused vitreous ceramic containing substantial proportions of boron, lead and lithium substances and having a metallic insert therein held in the article by the ceramic bond.

14. An abrasive article of the character described consisting of from 99.1% to 28.7% by weight of abrasive particles bonded with .9% to 71.3% by weight of fused vitreous ceramic containing substantial proportions of boron, lead and lithium substances.

KELSEY I. HARVEY.